

1

2,990,350

## RADIATION OF LUBRICATING OILS

Alvin M. Natkin, Metuchen, John J. Kolfenbach, North Plainfield, and Eric O. Forster, Scotch Plains, N.J., assignors to Esso Research and Engineering Company, a corporation of Delaware

No Drawing. Filed Mar. 1, 1956, Ser. No. 568,710

4 Claims. (Cl. 204—158)

This invention relates to lubricating oils, and more particularly to a process for improving the physical properties of lubricating oils. In brief compass, the invention pertains to obtaining improved lubricating oils by subjecting the lubricating oils to high intensity ionizing radiation.

In the prior art, when it has been desirable to improve the physical properties of lubricating oils special refining methods or additives have been employed. For example, higher viscosity indices of lubricating oils, i.e. the relative degree of change in the viscosity of the oils with respect to temperature changes, have been obtained by means of solvent refining methods or by means of special additives such as polybutene or other high molecular weight polymers.

In accordance with the present invention, it has now been found that lubricating oils having higher viscosity indices as well as other improved characteristics, such as viscosity, color, etc., can be obtained by subjecting the oils to high intensity ionizing radiation. In general, the lubricating oils are irradiated with gamma rays. These gamma rays may be derived from the radioactive decay of certain natural or radioactive elements or isotopes, such as radium 226, radium A, radium B, radium C, radium D, thallium 210, cobalt 60, cesium 137, europium 152—154, cesium 134, cerium 144, silver 110, thulium 170, tantalum 182, scandium 46, terbium 160, or iridium 192, or from chemical compounds of or materials containing such elements or isotopes. The gamma rays may also be derived from suitably shielded radiation produced in nuclear reactors, i.e. atomic piles, or from the spent fuel elements obtained from the operation of such reactors.

In general, undisturbed gamma ray fluxes within the range of about  $10^3$  to  $6 \times 10^8$ , usually about  $10^4$  to  $3 \times 10^8$ , roentgens per hour, such as that derived from a cobalt 60 source, will be employed in irradiating the lubricating oils of the invention. The time of irradiation will depend upon the degree of change in the physical properties of the lubricating oils desired as well as upon the radiation dosage rate. Generally, the total radiation dosage (based on undisturbed radiation field conditions, i.e. conditions prior to the introduction of the lubricating oil into the radiation field) will be within the range of about  $10^5$  to  $3 \times 10^{10}$ , preferably about  $10^6$  to  $3 \times 10^9$ , roentgens of gamma rays. Thus, irradiation time may vary from about 0.01 to 3000 hours, usually about 0.5 to 200 hours. For the purposes of this invention, however, the lubricating oil feed stocks may be irradiated for the shortest period of time required to obtain the desired viscosity indices and viscosities.

The lubricating oils may also be irradiated in an atomic pile wherein the radiation will consist primarily of fast and slow neutrons and gamma rays. Although there are some beta rays existing in the atomic piles, they are relatively insignificant since it appears that they are gen-

2

erally absorbed in the reactor. The slow neutrons are generally considered to be those neutrons having an energy less than about 30 electron volts (e.g. 0.03 electron volt), and the slow neutron flux in the atomic pile will be in the range of about  $10^9$  to  $10^{16}$ , usually about  $10^{11}$  to  $10^{15}$ , neutrons/cm.<sup>2</sup>/sec. The gamma ray flux will generally be about  $10^3$  to  $6 \times 10^8$ , usually about  $10^4$  to  $3 \times 10^8$  roentgens per hour. The radiation of an atomic pile will also contain a certain amount of fast neutrons having an undisturbed flux of about  $10^{10}$  to  $10^{17}$ , usually about  $10^{11}$  to  $10^{16}$  neutrons/cm.<sup>2</sup>/sec.

Any of the known mineral or synthetic lubricating oil base stocks may be employed as the feed material in the invention. In general, these lubricating oils should have a viscosity of about 10 to 2,000, preferably about 20 to 1,000 centistokes at 100° F. and about 1 to 100, preferably about 2 to 50 centistokes at 210° F., an A.S.T.M. pour point of about +40 to —75° F., a flash point of about 300° to 650° F., and a viscosity index of about 0 to 175, preferably about 20 to 160. Mineral lubricating oil base stocks derived from paraffinic, naphthenic and mixed base crudes having the properties listed above are especially useful in preparing the improved lubricating oils of the invention. As hereinafter shown, however, the phenol-treated naphthenic base lubricating oils are particularly preferred in that they show the most improvement in physical properties with little or no deleterious effects when subjected to irradiation.

The synthetic lubricating oils which may also be employed include esters of monobasic acids (e.g. an ester of C<sub>8</sub> Oxo alcohol with C<sub>8</sub> Oxo acid, an ester of C<sub>13</sub> Oxo alcohol with octanoic acid, etc.), esters of dibasic acids (e.g. di-2-ethyl hexyl sebacate, di-nonyl adipate, etc.), esters of glycols (e.g. C<sub>13</sub> Oxo acid diester of tetraethylene glycol, etc.), complex esters (e.g. the complex ester formed by reacting one mol of tetraethylene glycol with two moles of sebacic acid and two moles of 2-ethyl-hexanol, or the complex ester formed by reacting one mole of tetraethylene glycol, one mole of adipic acid, one mole of C<sub>8</sub> Oxo alcohol and one mole of C<sub>8</sub> Oxo acid, etc.), esters of phosphoric acid (e.g. the ester formed by contacting three moles of the mono-methyl ether of ethylene glycol with one mol of phosphorous oxychloride, etc.), halocarbon oils (e.g. the polymer of chlorotrifluoroethylene containing twelve recurring units of chlorotrifluoroethylene), carbonates (e.g. the carbonate formed by reacting C<sub>8</sub> Oxo alcohol with ethyl carbonate to form a half ester and reacting this half ester with tetraethylene glycol), mercaptals (e.g. the mercaptal formed by reacting 2-ethyl hexyl mercaptan with formaldehyde), formals (e.g. the formal formed by reacting C<sub>13</sub> Oxo alcohol with formaldehyde), poly-glycol type synthetic oils (e.g. the compounds formed by condensing butyl alcohol with fourteen units of propylene oxide, etc.), or mixtures of the above in any proportions.

The irradiation of the lubricating oil feed stock may be carried out by a variety of procedures. For example, the radioactive source may be placed in a tank containing a suitable lubricating oil to carry out a batch operation or the radioactive source may be placed into a stream of such lubricating oil to carry out a continuous process. The lubricating oil may also be piped through an atomic reactor or pile as a continuous stream wherein the oil is exposed to the neutrons and gamma rays. Many obvious modifications of these procedures will be

apparent to those skilled in the art. The utilization of radiation emitted by radioactive materials necessitates, of course, the provision of adequate radiation shielding means and techniques. Such means and techniques are, however, well known in the art and need not be described herein in detail.

The irradiation of the lubricating oils may generally be carried out at temperatures within the range of about -20° to 400° F. or higher. Ordinarily, the irradiation will be carried out at a temperature of about 50° to 10 200° F., preferably about 70° to 150° F., and under vacuum or elevated pressures, such as about 2 to 50 atmospheres. However, one of the advantages of the present process is that it may be effectively utilized at room temperatures and at atmospheric pressure. If car-

5 15 (5) Lubricating Oil E—A phenol-treated naphthenic type oil having a viscosity of 20.5 cs. at 100° F. and 3.7 cs. at 210° F., 54.3 V.I., an API gravity of 28.9°, a flash point of about 340° F. and a pour point of about -50° F. This lubricating oil was derived from a Coastal crude.

(6) Lubricating Oil F—A paraffinic type oil having a viscosity of 86.0 cs. at 100° F. and 10.0 cs. at 210° F., 104.8 V.I., an API gravity of 30.2°, a flash point of about 485° F. and a pour point of about +20° F. This lubricating oil was derived from a Mid-Continent crude.

(7) Lubricating Oil G—A synthetic oil comprising C<sub>13</sub> Oxo formal having a viscosity of 16.0 cs. at 100° F. and 3.60 cs. at 210° F.

The inspections of the irradiated lubricating oils are set forth in the table below:

Table I

EFFECT OF  $\gamma$ -RADIATION ON LUBRICATING OILS

| Lubricating Oil | Viscosity, Centistokes |         |                  |            |       |                  | V.I.   |       |                  | Neut. No. |       | Change In Color |                  |
|-----------------|------------------------|---------|------------------|------------|-------|------------------|--------|-------|------------------|-----------|-------|-----------------|------------------|
|                 | at 100° F.             |         |                  | at 210° F. |       |                  | Before | After | Percent Increase | Before    | After | Before          | After            |
|                 | Before                 | After   | Percent Increase | Before     | After | Percent Increase | Before | After | Percent Increase | Before    | After | Before          | After            |
| A-----          | 198.8                  | 250.2   | 25.8             | 12.5       | 14.4  | 15.2             | 36.1   | 36.3  | 0.5              | 0.04      | 0.08  | Reddish brown.  | Reddish yellow.  |
| B-----          | 857.0                  | 1,165.0 | 26.4             | 39.6       | 49.2  | 24.2             | 87.5   | 90.2  | 3.1              | 0.19      | 0.19  | Greenish black. | Greenish black.  |
| C-----          | 12.7                   | 21.4    | 68.6             | 3.4        | 4.8   | 42.3             | 156.1  | 159.0 | 1.8              | 0.12      | 0.21  | Colorless.      | Colorless.       |
| D-----          | 268.3                  | 344.0   | 28.4             | 14.9       | 17.5  | 17.5             | 34.2   | 38.6  | 12.8             | 0.03      | 0.02  | Greenish brown. | Greenish yellow. |
| E-----          | 20.5                   | 25.5    | 25.1             | 3.7        | 4.3   | 14.8             | 54.3   | 61.0  | 12.5             | 0.06      | 0.02  | Yellow brown.   | Straw yellow.    |
| F-----          | 86.0                   | 112.5   | 30.8             | 10.0       | 12.3  | 22.3             | 104.8  | 107.2 | 2.3              | 0.06      | 0.12  | Yellow red.     | Yellow.          |
| G-----          | 16.14                  | 20.40   | 27.0             | 3.60       | 4.23  | 17.0             | 120.3  | 129.3 | 7.6              | 0.03      | 30.53 |                 |                  |

bonaceous solids or hydrocarbon materials having boiling points outside of the lubricating oil boiling range, e.g. higher boiling polymeric material or lower boiling hydrocarbons; are formed the irradiated lubricating oil may be recovered by any of the conventional methods, e.g. filtration, distillation, etc.

The following examples and tables are presented to illustrate the preparation and the various characteristics of the improved lubricating oils of the invention.

## EXAMPLE I

A number of lubricating oils were irradiated by filling one ounce screw-top bottles to the neck with the lubricating oil, closing the bottle with a plastic screw-top to leave very little air in the container, and then lowering the bottles into the center of a cylindrical cobalt 60 source. The undisturbed radiation intensity of this source was about  $2.2 \times 10^8$  roentgens/hour. The following lubricating oil samples were exposed to radiation of this intensity for 168 hours:

(1) Lubricating Oil A—An acid-treated naphthenic type oil having a viscosity of 198.8 cs. at 100° F. and 12.5 cs. at 210° F., 36.1 V.I., an API gravity of 22.4°, a flash point of about 440° F. and a pour point of about -15° F. This lubricating oil was derived from a Coastal crude.

(2) Lubricating Oil B—A paraffinic type oil having a viscosity of 857 cs. at 100° F. and 39.6 cs. at 210° F., 87.5 V.I., an API gravity of 22.0°, a flash point of 560° F. and a pour point of +25° F. This lubricating oil was derived from a Mid-Continent crude residuum.

(3) Lubricating Oil C—A synthetic ester comprising di-2-ethylhexyl sebacate having a viscosity of 12.7 cs. at 100° F. and 3.4 cs. at 210° F. and a 156 V.I.

(4) Lubricating Oil D—A phenol-treated naphthenic type oil having a viscosity of 268.3 cs. at 100° F. and 14.9 cs. at 210° F., 34.2 V.I., an API gravity of 22.2°, a flash point of about 440° F. and a pour point of about 0° F.

40

The above data show that the high intensity gamma ray irradiation of lubricating oils will result in marked changes in the physical properties of the lubricating oils. The data further show that paraffinic type mineral lubricating oils are less susceptible to change in certain properties by irradiation than the naphthenic type mineral lubricating oils, particularly the phenol-treated naphthenic oils, while the synthetic type lubricating oils are the most affected. It should be noted, however, that the synthetic lubricating oils, as represented by Lubricating Oil C, show a very large increase in their neutralization number in contrast to the mineral lubricating oils which do not show any change at all in this respect.

The lubricating oils produced in accordance with the present invention may be employed in lubricating oil compositions and in lubricating grease compositions. Furthermore, the lubricating oils of the present invention may have minor proportions of conventional lubricant additives incorporated therein. More particularly, the lubricating oils may contain detergents (e.g. barium nonyl phenol sulfide, calcium sulfonates), oxidation inhibitors (e.g. phenyl alpha-naphthylamine; di-tertiary butyl paracresol), corrosion inhibitors (e.g. zinc dihexyl dithiophosphate), rust inhibitors, dyes, anti-foaming agents, etc. The lubricating grease compositions may contain conventional grease thickeners such as fatty acid soaps (e.g. calcium stearate), soap-salt or mixed salt complex thickeners (e.g. calcium acetate-calcium stearate), polyethylene, polybutene, silica gel, carbon black, etc. as well as the conventional inhibitors listed above.

In accordance with one aspect of this invention, however, it is important not to have the conventional additives present during irradiation. As shown in the following example, the presence of conventional oxidation inhibitors during irradiation will result in a loss of their effectiveness as antioxidants and, in some instances, will minimize the changes in the physical properties of the lubricating oils.

75

## EXAMPLE II

The following lubricating oils and the lubricating oil compositions were irradiated in a manner similar to that of Example I except that field intensity was  $1.74 \times 10^6$  roentgens per hour:

Table II

| Lubricant                             | Micro Viscosity, Cs. |         | Neut. No. | Alcoa Oxidation Life, Hrs. <sup>1</sup> |
|---------------------------------------|----------------------|---------|-----------|-----------------------------------------|
|                                       | 100° F.              | 210° F. |           |                                         |
| Lubricating Oil F:                    |                      |         |           |                                         |
| Before                                | 86.65                | 9.987   | 0.01      | 30                                      |
| After                                 | 111.60               | 11.94   | 0.01      | 28                                      |
| Lubricant Composition R: <sup>2</sup> |                      |         |           |                                         |
| Before                                | 86.03                | 9.90    | 0.05      | 90                                      |
| After                                 | 98.09                | 10.89   | 0.01      | 27                                      |
| Lubricant Composition S: <sup>3</sup> |                      |         |           |                                         |
| Before                                | 86.29                | 9.92    | 0.05      | 360                                     |
| After                                 | 112.80               | 12.07   | 0.02      | 20                                      |
| Lubricating Oil H: <sup>4</sup>       |                      |         |           |                                         |
| Before                                | 91.03                | 8.586   | 0.05      | 25                                      |
| After                                 | 111.70               | 9.808   | 0.04      | 27                                      |
| Lubricant Composition T: <sup>5</sup> |                      |         |           |                                         |
| Before                                | 89.97                | 8.538   | 0.15      | 40                                      |
| After                                 | 118.0                | 9.951   | 0.12      | 12                                      |
| Lubricant Composition U: <sup>6</sup> |                      |         |           |                                         |
| Before                                | 22.35                | 3.633   | 0.05      | -----                                   |
| After                                 | 23.07                | 3.906   | 0.02      | -----                                   |

<sup>1</sup> Time to 60 mm. Hg pressure drop.

<sup>2</sup> Lubricating Oil F plus 0.8 wt. percent Oxidation Inhibitor A and 0.05 wt. percent Rust Inhibitor A.

<sup>3</sup> Lubricating Oil F plus 0.4 wt. percent Oxidation Inhibitor B and 0.05 wt. percent Rust Inhibitor A.

<sup>4</sup> A phenol-treated naphthenic lubricating oil having a viscosity of 55 SUS at 210° F.

<sup>5</sup> Lubricating Oil H plus 0.4 wt. percent Oxidation Inhibitor A and 0.075 wt. percent Rust Inhibitor B.

<sup>6</sup> An acid-treated naphthenic lubricating oil having a viscosity of 40 SUS at 210° F. plus 0.4 wt. percent Oxidation Inhibitor B, 0.2 wt. percent Oxidation Inhibitor A and 0.05 wt. percent Rust Inhibitor A.

It will be further understood that the invention is not necessarily limited to the specific materials and operating conditions of the foregoing examples. These materials and conditions may be varied within the limits indicated in the general portions of the specification.

What is claimed is:

1. A method of increasing the viscosity and viscosity

index of a lubricating oil which comprises exposing a lubricating oil having initially a viscosity in the range of 10 to 2000 cs. at 100° F., a pour point in the range of +40° to -75° F., and a flash point in the range of 300° to 650° F., to gamma irradiation until in the range of  $10^6$  to  $3 \times 10^8$  Roentgens of energy have been absorbed, and recovering a lubricating oil product having an increased viscosity and viscosity index.

2. The method of claim 1 wherein the gamma dosage is in the range of  $10^4$  to  $3 \times 10^8$  Roentgens per hour.

3. A method of increasing the viscosity and viscosity index of a naphthenic lubricating oil which comprises exposing a naphthenic base lubricating oil having initially a viscosity in the range of 10 to 2000 cs. at 100° F., a pour point in the range of +40° to -75° F., and a flash point in the range of 300° to 650° F., to gamma irradiation at a temperature in the range of -20° to 400° F. until in the range of  $10^6$  to  $3 \times 10^8$  Roentgens of energy have been absorbed, and recovering a lubricating oil product having an increased viscosity and viscosity index.

4. A method comprising exposing a phenol treated naphthenic type oil having initially a viscosity of 14.9 cs. at 210° F., a viscosity index of 34.2, and an API gravity of 22.2°, a flash point of about 440° F., and a pour point of about 0° F., to gamma irradiation obtained from cobalt 60 at a dosage of about  $2.2 \times 10^6$  Roentgens per hour for 168 hours, and recovering an improved product having a viscosity of 17.5 cs. at 210° F. and a viscosity index of 38.6.

30

## References Cited in the file of this patent

## FOREIGN PATENTS

697,601 Great Britain ----- Sept. 23, 1953

## OTHER REFERENCES

Relative Merits of Cathode Rays and Gamma Radiations, by Goldblith and Proctor, from Nucleonics, February 1954, vol. 12, No. 2, pp. 32-35.

Radiation Stability of Plastics and Elastomers, by Bopp & Sisman, from Nucleonics, vol. 13, No. 7, July 1955, pp. 28-33.

35